

Oct. 30, 1962

H. BOGATY ET AL

3,060,551

MIXED FABRIC WITH WOOL SURFACE

Filed Aug. 11, 1959.



WARP



FILLING

INVENTORS

*Herman Bogaty,  
Norman R.S. Hollies,  
John C. Hintermaier.*

BY

*H. J. Euston.*

ATTORNEY

# United States Patent Office

**3,060,551**

Patented Oct. 30, 1962

1

3,060,551

**3,000,331**  
**MIXED FABRIC WITH WOOL SURFACE**

**MAILED PARCELS WITH WIRE SEALS**  
**Herman Bogaty, Evanston, Ill., Norman R. S. Hollies,**  
**Bethesda, Md., and John C. Hintermaier, Troy, N.Y.,**  
**assignors to the United States of America as repre-**  
**sented by the Secretary of the Army**

Filed Aug. 11, 1959, Ser. No. 833,117  
16 Claims. (Cl. 28—78)

This invention relates to a mixed wool and artificial fiber fabric having wearing characteristics substantially equivalent to an all-wool fabric.

A neat military appearance is a strong morale factor among the troops in the field. There are two aspects of appearance: the garment must meet reasonably high standards of appearance after tailoring; and the garment must continue to present a suitable appearance after continued wear, pressing and cleaning. Wool garments meet these standards and additionally they exhibit desirable attributes of comfort, particularly for cold weather wear. While the comfort characteristics of wool clothing are not completely understood, the advantages of fabrics made entirely or substantially of wool are thought to stem *inter alia* from the resiliency of the wool fiber, the capacity of wool to absorb water vapor transpired by the skin, and the resistance of wool cloth to transfer of liquid water by "wicking." Additional important virtues of wool fabrics for warmth and comfort are believed to be derived from the typical "hairiness" of the wool fabric surface: the tendency for wool fabrics to be bulky for their weight and hence, to exhibit effective thermal insulation, to resist wetting of the surface by liquid water, to yield to compression of the thickness but to recover its original thickness on removal of the compressive forces and to feel warm to the touch. Wool garments normally meet the standards of appearance and the wearing and comfort characteristics described but wool is scarce during wartime and its procurement is a substantial cost item even in time of peace.

The United States Army has adopted a flannel-type mixed wool and nylon fabric consisting of about 85% wool and about 15% nylon. Such a fabric is specified in Military Specification MIL-C-11065A (QMC) Cloth, Wool and Nylon, Flannel, 16 Ounce, Shrink Resistant, 27 June 1958. This fabric has very favorable wearing characteristics, but effects a saving of only about 15% wool.

A larger reduction of the wool content of a mixed wool and synthetic fabric without impairment of wearing characteristics, is desirable for military and civilian uses, inasmuch as wool is a critical commodity during times of national emergency. While fabrics containing 30-50% of synthetic fibers in admixture with wool have been produced by others, these fabrics tend to be thin and hence, poor thermal insulators. They are cool to the touch, easily wet by water, and low in water vapor absorption in many cases. The present invention provides a

means to achieve reduction of wool content in mixed wool and synthetic fabrics without material impoverishment of the desirable wool-like characteristic of the cloth.

5 By 1945, when clothing made of 100% wool and  
about 30-50% crimped, short-staple artificial fibers and  
selection of appropriate warp and filling yarns, fabric  
construction and shrinkage factors, there is produced a  
lofty fabric with a nearly "all-wool" surface, wherein  
the artificial fibers component remain principally im-  
10 bedded in the interior. This fabric can be produced at  
substantially less cost than the 85% wool, 15% nylon  
fabric now in military use. Our tests have shown the  
suitability of a very wide variety of artificial man-made  
fibers in crimped short staple form for random admix-  
15 ture with wool in the production of yarns for the purposes  
of our invention. Such fibers include, but are not limited  
to the following:

TABLE I

|    |                                |                                                                                                                                             |
|----|--------------------------------|---------------------------------------------------------------------------------------------------------------------------------------------|
| 20 | Commercial name:<br>Nylon----- | Chemical composition<br>Long-chain oriented synthetic poly-<br>amide, e.g., hexamethylene adip-<br>amide polymer or caprolactam<br>polymer. |
| 25 | Viscose-----                   | Regenerated cellulose (rayon).                                                                                                              |
|    | Acetate-----                   | Cellulose acetate.                                                                                                                          |
|    | Dynel-----                     | Vinyl chloride and acrylonitrile<br>copolymer.                                                                                              |
|    | Vinyon N-----                  | Do.                                                                                                                                         |
| 30 | Dacron-----                    | Ethylene glycol and terephthalic<br>acid polyester.                                                                                         |
|    | Orlon-----                     | Polyacrylonitrile.                                                                                                                          |
|    | Acrilan-----                   | Mixed polymer (about 85% acryloni-<br>trile and about 15% vinyl deriva-<br>tives).                                                          |
| 35 | Vicara-----                    | Regenerated protein fiber from zein.                                                                                                        |

Performance testing has led us to the conclusion that ternary yarns, i.e., yarns composed of wool fibers and two different artificial fibers, give the best results because of greater latitude in selection; however, a number of binary yarns, i.e., yarns composed of wool fibers and one artificial fiber, may be employed for the purposes of our invention. A typical ternary yarn for the practice of our invention may be composed e.g., of 65-70% wool fibers, 10-15% nylon crimped short staple fibers and 20-25% rayon (viscose) crimped short staple fibers. Best results in terms of fabric performance were obtained with ternary yarns composed of 65% wool fibers (e.g., 40% wool tops and 25% wool noils), 15% nylon crimped short staple fibers and 20% rayon (viscose) or dynel crimped short staple fibers; another ternary yarn giving very favorable results when woven in accordance with the present invention is composed of 65% wool fibers, 20% dynel crimped short staple fibers and 15% rayon (viscose) crimped short staple fibers.

Other mixed yarn combinations suitable for producing a mixed fabric in accordance with our invention are, e.g.:

TABLE 2

| Wool,<br>percent | Vicara,<br>percent | Viscose,<br>percent | Nylon,<br>percent | Dynel,<br>percent | IIS (high<br>shrink),<br>percent | Dynel<br>percent | Orlon,<br>percent | HS (high<br>shrink),<br>percent | Orlon<br>percent |
|------------------|--------------------|---------------------|-------------------|-------------------|----------------------------------|------------------|-------------------|---------------------------------|------------------|
| 70               | 15                 |                     | 15                |                   |                                  |                  |                   |                                 |                  |
| 70               |                    | 20                  | 10                |                   |                                  |                  |                   |                                 |                  |
| 70               |                    | 30                  |                   |                   |                                  |                  |                   |                                 |                  |
| 70               |                    |                     |                   | 30                |                                  |                  |                   |                                 |                  |
| 65               |                    | 20                  | 15                |                   |                                  |                  |                   |                                 |                  |
| 65               |                    | 15                  |                   | 20                |                                  |                  |                   |                                 |                  |
| 65               |                    |                     | 15                | 20                |                                  |                  |                   |                                 |                  |
| 60               |                    | 20                  |                   |                   |                                  |                  | 20                |                                 |                  |
| 60               |                    | 20                  |                   | 20                |                                  |                  |                   |                                 |                  |
| 50               |                    | 35                  | 15                |                   |                                  |                  |                   |                                 |                  |
| 50               |                    |                     |                   | 15                | 35                               |                  |                   |                                 |                  |
| 50               |                    |                     | 15                |                   |                                  |                  |                   | 35                              |                  |
| 50               |                    |                     |                   |                   |                                  |                  | 15                | 35                              |                  |

The foregoing table shows the viscose (regenerated cellulose rayon) fiber content of mixed yarns suitable for the purpose of our invention to be as low as 0% and as high as 35% of the total fiber content.

It will be understood, of course, that fabrics produced in accordance with our invention from these mixed yarns somewhat differ from each other in performance characteristics e.g., with regard to tensile strength, abrasion strength, thermal insulation, water absorption, etc.; however, they are all "wool-plated" in the sense that the surface cover of the fabric consists of fibers projecting from the surface of the cloth which projecting fibers are mainly wool fibers, while the synthetic fibers remain for the most part embedded in the interior of the fabric, whereby the wearer of the garment is given the feeling of wearing an all-wool garment.

It accordingly is an object of the present invention to provide a mixed wool fabric having wearing and comfort characteristics at least equivalent to an all-wool fabric, and containing a larger percentage of artificial fibers than heretofore practiced by the art.

Another object of the invention is a mixed wool and artificial fabric having a nearly all-wool surface and wherein the artificial fibers are principally in the interior of the fabric.

A further object of our invention is a mixed wool and synthetic fabric which can be woven on conventional weaving machinery, and which is subsequently processed by methods familiar to those working in the art.

Other objects and advantages, will become apparent from the following description of the principles on which the invention is based and of a preferred mode of carrying the same into practice.

As stated, our invention produces a fabric which is "wool-plated" on its surface even when up to 50% of the wool is replaced by a synthetic fiber of suitable diameter and staple length. The invention utilizes the differential migration qualities of wool and artificial fibers during fulling to produce a lofty fabric with good surface wool cover.

Garments that may be made from such fibers include, e.g., shirts, trousers, jackets; of the foregoing uses, the one presently considered to be of principal importance is as a shirting fabric. The surface wool cover of the shirting and other fabrics made in accordance with our invention is produced without resorting to the mechanical process commonly used in industry of brushing the fabric with wire brushes, raising fibers from the surface of the fabric to produce a nap (a process commonly known as napping). Our fabric is engineered to maximize the differential shrinkage properties of the fibers and the tendency of wool fibers to migrate during fulling by utilizing a loose construction throughout the preliminary stages of manufacturing. The loose construction promoted freedom of motion for the fiber during the fulling operation. Without necessarily limiting ourselves to the following enumeration, we presently conclude that the desirable "wool-plating" effect of the fabrics produced in accordance with our invention, is due to a combination of the following features:

(1) Selection of diameter and length of synthetic fiber to blend with wool. In general, thicker, shorter crimped synthetic fibers are used in the practice of this invention than is commonly practiced by the industry.

(2) The yarns are spun with a low twist. The level of twist is approximately two-thirds that normally used by the industry for the same count yarn.

(3) A coarser yarn is used in the filling than in the warp.

(4) Opposing twists are used in warp and filling yarns.

(5) A loose weave is used such as a 3/1 crowfoot, or other satin or twill weaves (e.g. 2/2 common twill) having relatively long floats (2 or more) consistent with a loose fabric construction.

(6) Length shrinkage in fulling is about 20-30%, e.g.,

25%, which differs from common practice to 10-15% fulling shrinkage. In other words, our fabric is shrunk to about 70-80% of (preferably about 75%) its original length during fulling.

We recommend in the manufacture of the fabric that the warp is reeded wide in the loom, e.g., 72 inches or wider for a 56" finished width, and that a low number of picks is used in the loom.

In the appended drawings there is illustrated in diagrammatic form a typical fabric in accordance with our invention.

FIGURE 1 is a schematic transverse section, in greatly enlarged scale, through a 3/1 crowfoot satin fabric produced in accordance with our invention; and

FIGURE 2 is a diagrammatic weave chart of a 3/1 crowfoot warp face satin fabric at a still larger scale.

FIGURE 1 shows warp yarn 11 floated over three filling yarns 12; a fuzzy surface cover 13, 13', almost entirely wool, constitutes the top and bottom surfaces of the fabric, while the artificial fiber components of the mixed wool and artificial fiber warp and filling yarns remain the interior of the fabric.

In conformance with the patent statutes, we now proceed to a manufacturing description of the production of a preferred 16 ounce shirting fabric, in accordance with our invention, without, of course, restricting the scope of our invention to any specific technical details set forth.

#### Example 1

Yarn: 40% wool tops and 25% wool noils, 20% viscose (rayon) and 15% nylon.

Wool tops: Grade 58/60's Super A grade pulled or fleece (USDA grade) carbonized.

Wool noils: Grade 60/62's (USDA grade), carbonized.

Viscose: 5.5 denier, delustered, crimped, 1½" staple.

Nylon: 6 denier, 1½" staple, crimp set.

Weave loose crowfoot satin 3/1, warp face.

Width, exclusive of selvage 56".

Thread count per inch in finished cloth: 38 warp, 33 filling.

Yarn size, nominal, warp 3½ run, filling 3¼ run (filling yarn slightly coarser than warp yarn).

Yarn twist per inch, nominal, warp S 8.5 to 9, filling Z 7.5 to 8 (opposite twist).

Reed width: 72" for a 56" fabric. Width of gray goods: 65-68".

The goods are fulled by heat and moisture to a width of about 56", and to a length shrinkage of about 9" per yard (corresponding to a length reduction of about 25%).

A conventional shrink resistant treatment, e.g., commercial chlorination or resin treatment may be applied. Olive drab color is suitable for military shirting.

Other weaves made in the same manner had the following structures:

|                                         | Example 2 |      | Example 3 |      | Example 4 |      | Example 5 |      |
|-----------------------------------------|-----------|------|-----------|------|-----------|------|-----------|------|
|                                         | Warp      | Fill | Warp      | Fill | Warp      | Fill | Warp      | Fill |
| 60                                      |           |      |           |      |           |      |           |      |
| Thread count per inch in finished cloth | 40.0      | 36.0 | 40.0      | 38.0 | 39.0      | 37.0 | 35.0      | 30.0 |
| Yarn size (runs)                        | 3.10      | 2.70 | 3.20      | 2.90 | 3.25      | 3.00 | 3.00      | 2.80 |
| Yarn twist (per inch)                   | 10 S      | 9 Z  | 9½ S      | 8½ Z | 8½ S      | 7½ Z | 8 S       | 7 Z  |

It will thus be seen that we have provided an open weave mixed wool and artificial fiber fabric of excellent military and civilian wearing characteristics, which is characterized by random distribution of the wool and artificial fibers, by a lofty bulkiness and by a hairy wool surface cover on both sides, while the artificial fibers remain principally embedded in the interior of the fabric.

The fabric possesses water resistance substantially equal to the water resistance of an all-wool fabric, and a strength at least equal to that of an all-wool fabric. Our fabric is preferably composed of warp and filling yarns of opposite low-twist, the filling yarns being slightly coarser than the warp yarns. The wool component of our fabric yarns is 50-70% wool fibers and randomly distributed therewith artificial 30-50% crimped short staple fibers, of which we prefer at least 10-15% to be nylon or dynel fibers. Our fabric construction is a loose long-float weave, fulled so as to shrink the fabric to about 70-80% of its original unfulled length. Such "wool-plated" mixed fabrics are suitable for military and civilian garments customarily made of all-wool materials, such as shirts, trousers, jackets, etc. and are their functional equivalents or even superiors, if the principles of our invention are observed in manufacturing.

The thickness or loftiness obtained in this fabric is shown in the following table, which also shows the thicknesses for several variations of fiber composition, otherwise made in the same way.

TABLE 3

| Composition:                         | Thickness at 0.01 p.s.i. in inches |
|--------------------------------------|------------------------------------|
| Wool 65%, rayon 20%, nylon 15% ----- | .114                               |
| Wool 65%, rayon 15%, dynel 20% ----- | .104                               |
| Wool 65%, nylon 15%, dynel 20% ----- | .106                               |

The measurement of thickness is taken on relaxed fabric, that is, fabric which has been wet out and allowed to dry without pressure or tension on a flat surface. The measurement was made with the Schiefer compressometer, using a disc five inches in diameter. The operation of the Schiefer compressometer is described in the National Bureau of Standards Journal of Research, vol. 10 (1933), pages 705-713.

By comparison, thickness measurements on twenty samples of 85% wool, 15% nylon shirting fabrics, in accordance with the military specification identified in the third paragraph of the specification, averaged .1075 inch.

Having thus described the principles of our invention and several preferred modes of carrying the same into practice, it is evident that several modifications and adaptations will readily occur to the expert without departing from the essence of our invention. We therefore desire to encompass such modifications and adaptations within the scope of our invention, and to this end define the same by the appended claims.

We claim:

1. A mixed wool and artificial fiber fabric having wearing characteristics substantially equivalent to an all-wool fabric, said fabric having warp and filling yarns of low twist, said yarns being composed of about 50-70% wool fibers and about 30-50% crimped short staple artificial fibers in random distribution, said yarns including in their artificial fiber component about 0-35% cellulosic fibers, and said warp and filling yarns being woven into a loose weave having warp yarn floats over at least 2 filling yarns, said loose fabric being shrunk to about 70-80% of its original length, whereby a lofty resilient fabric with a wool surface cover is produced and wherein the artificial fibers remain principally embedded in the interior of said fabric.

2. A mixed wool and artificial fiber fabric having wearing characteristics substantially equivalent to an all-wool fabric, said fabric having warp and filling yarns of opposite low twist, said yarns being composed of about 50-70% wool fibers and about 30-50% crimped short staple artificial fibers in random distribution, said yarns including in their artificial fiber component about 0-35% cellulosic fibers, and said warp and filling yarns being woven into a loose weave having warp yarn floats over at least 2 filling yarns, said loose fabric being shrunk to about 70-80% of its original length, whereby a lofty resilient fabric

with a wool surface cover is produced and wherein the artificial fibers remain principally embedded in the interior of said fabric.

3. A mixed wool and artificial fiber fabric having wearing characteristics substantially equivalent to an all-wool fabric, said fabric having warp and filling yarns of low twist, said yarns being composed of about 50-70% wool fibers and about 30-50% crimped short staple artificial fibers in random distribution, said yarns including in their artificial fiber component about 0-35% cellulosic fibers, said filling yarns being slightly coarser than said warp yarns, and said warp and filling yarns being woven into a loose weave having warp yarn floats over at least 2 filling yarns, said loose fabric being shrunk to about 70-80% of its original length, whereby a lofty resilient fabric with a wool surface cover is produced and wherein the artificial fibers remain principally embedded in the interior of said fabric.

4. Fabric according to claim 1, wherein said yarns contain about 65% wool fibers.

5. Fabric according to claim 1, wherein said yarns contain at least about 10% nylon fibers.

6. Fabric according to claim 1, wherein said yarn is composed of about 65% wool fibers, about 20% rayon fibers and about 15% nylon fibers.

7. Fabric according to claim 1, wherein said artificial fibers comprise vinyl chloride acrylonitrile copolymer fibers.

8. Fabric according to claim 1, wherein said artificial fibers comprise polyacrylonitrile fibers.

9. Fabric according to claim 1 wherein said yarn is composed of about 65% wool fibers, about 15% rayon and about 20% vinyl chloride acrylonitrile copolymer fibers.

10. Fabric according to claim 1 wherein said yarn is composed of about 65% wool fibers, about 15% nylon and about 20% vinyl chloride acrylonitrile copolymer fibers.

11. Fabric according to claim 1 wherein said yarn is composed of about 70% wool fibers, about 15% nylon and about 15% regenerated zein protein fibers.

12. Fabric according to claim 1, wherein said loose weave is a satin-type weave having warp yarn floats over at least 3 filling yarns.

13. A mixed wool-nylon-rayon fiber fabric having wearing characteristics substantially equivalent to an all-wool fabric, said fabric having warp and filling yarns of opposite low twist of from about 7 to about 10 turns per inch, said filling yarns having a slightly lower twist than 50 and being somewhat coarser than said warp yarns, said warp and filling yarns being composed of about 50-70% wool fibers and about 30-50% crimped short staple nylon and rayon fibers including at least about 10% nylon fibers in random distribution, and being woven into a loose 3/1 55 crowfoot satin weave, said loose fabric being shrunk to about 70-80% of its original length, whereby a lofty resilient fabric with a wool surface cover is produced and wherein the nylon and rayon fibers remain principally embedded in the interior of said fabric.

14. Fabric according to claim 13, wherein said warp and filling yarns contain about 65% wool fibers, about 15% nylon fibers and about 20% rayon fibers.

15. Fabric according to claim 14, wherein said wool fibers include about 40% wool tops and about 25% wool noils.

16. A mixed wool and artificial fiber fabric having wearing characteristics substantially equivalent to an all-wool fabric, said fabric having warp and filling yarns of low twist, said yarns being composed of about 65-70% 70 wool fibers and about 30-35% crimped short staple artificial fibers including at least about 10% non-cellulosic fibers, in random distribution, and said warp and filling yarns being woven into a loose weave having warp yarn floats over at least 2 filling yarns, said loose fabric being shrunk to about 70-80% of its original length, whereby a

lofty resilient fabric with a wool surface cover is produced and wherein the artificial fibers remain principally embedded in the interior of said fabric.

References Cited in the file of this patent

UNITED STATES PATENTS

2,125,925 Jones Aug. 9, 1938

|           |               |       | 8              |
|-----------|---------------|-------|----------------|
| 2,390,386 | Radford       | ----- | Dec. 4, 1945   |
| 2,407,602 | Cluley et al. | ----- | Sept. 10, 1946 |
| 2,586,538 | Speakman      | ----- | Feb. 19, 1952  |
| 2,686,538 | Nelson        | ----- | Aug. 17, 1954  |
| 2,792,851 | Moeckel       | ----- | May 21, 1957   |
| 2,897,042 | Heiks         | ----- | July 28, 1959  |
| 3,006,055 | Chapin        | ----- | Oct. 31, 1961  |

UNITED STATES PATENT OFFICE  
CERTIFICATE OF CORRECTION

Patent No. 3,060,551

October 30, 1962

Herman Bogaty et al.

It is hereby certified that error appears in the above numbered patent requiring correction and that the said Letters Patent should read as corrected below.

Column 2, "TABLE 2", the sixth and seventh column headings should appear as shown below instead of as in the patent:

HS (high  
shrink) Dynel  
percent

strike out the vertical line between the sixth and seventh columns; same TABLE 2, the ninth and tenth column headings, should appear as shown below instead of as in the patent:

HS (high  
shrink) Orlon  
percent

strike out the vertical line between the ninth and tenth columns; column 8, line 3, for "2,586,538" read  
-- 2,586,106 --.

Signed and sealed this 30th day of April 1963.

(SEAL)

Attest:

ERNEST W. SWIDER  
Attesting Officer

DAVID L. LADD  
Commissioner of Patent